



US007144613B2

(12) **United States Patent**  
Eguchi et al.

(10) **Patent No.:** US 7,144,613 B2  
(45) **Date of Patent:** Dec. 5, 2006

(54) **RECORDING MEDIUM, PROCESS FOR PRODUCTION THEREOF, AND INK-JET RECORDING METHOD EMPLOYING THE MEDIUM**

(75) Inventors: **Takeo Eguchi**, Tokyo (JP); **Kyo Miura**, Yokohama (JP); **Hitoshi Yoshino**, Zama (JP)

(73) Assignee: **Canon Kabushiki Kaisha**, Tokyo (JP)

(\*) Notice: Subject to any disclaimer, the term of this patent is extended or adjusted under 35 U.S.C. 154(b) by 0 days.

(21) Appl. No.: **08/974,513**

(22) Filed: **Nov. 19, 1997**

(65) **Prior Publication Data**

US 2001/0055055 A1 Dec. 27, 2001

**Related U.S. Application Data**

(63) Continuation of application No. 08/528,208, filed on Sep. 12, 1995, now abandoned.

(30) **Foreign Application Priority Data**

Sep. 16, 1994 (JP) ..... 6-221496  
Aug. 31, 1995 (JP) ..... 7-223694

(51) **Int. Cl.**  
**B41M 5/00** (2006.01)  
**B05D 5/04** (2006.01)

(52) **U.S. Cl.** ..... **428/32.37; 427/146; 427/372.2;**  
428/32.31; 428/32.15

(58) **Field of Classification Search** ..... 428/323,  
428/402, 195, 211, 537.5, 323.1, 32.37, 32.31  
See application file for complete search history.

(56) **References Cited**

U.S. PATENT DOCUMENTS

4,202,870 A 5/1980 Weber et al. ..... 423/630  
4,242,271 A 12/1980 Weber et al. ..... 260/448

|               |         |                      |           |
|---------------|---------|----------------------|-----------|
| 4,474,847 A   | 10/1984 | Schroder et al. .... | 428/323   |
| 4,879,166 A   | 11/1989 | Misuda et al. ....   | 428/212   |
| 4,946,666 A * | 8/1990  | Brown .....          | 423/625   |
| 5,104,730 A   | 4/1992  | Misuda et al. ....   | 428/304.4 |
| 5,122,814 A   | 6/1992  | Endo et al. ....     | 346/33 R  |

FOREIGN PATENT DOCUMENTS

|    |             |        |
|----|-------------|--------|
| DE | 3024205 A 1 | 1/1982 |
| EP | 0500021 A 1 | 8/1992 |

(Continued)

OTHER PUBLICATIONS

The Journal of the American Chemical Society vol. LXXIII, dated Jan.-Mar. 1951, pp. 373-380.

(Continued)

*Primary Examiner*—Pamela R. Schwartz

(74) *Attorney, Agent, or Firm*—Fitzpatrick, Cella, Harper & Scinto

(57) **ABSTRACT**

In a recording medium having a porous ink-receiving layer containing alumina hydrate of boehmite structure formed on a base material, the alumina hydrate has crystallinity ranging from 15 to 80 and microcrystals of the alumina hydrate are directed to be parallel to a plane direction of the ink-receiving layer at a parallelization degree of not less than 1.5. The recording medium is employed in an ink-jet recording method conducting printing by ejecting ink droplets through an orifice onto the recording medium.

A process for producing the recording medium comprises the steps of: applying a coating liquid containing alumina hydrate of boehmite structure with shearing stress onto a base material; and drying the coated material to obtain a degree of parallelization of a microcrystal of the alumina hydrate with a plane direction of the ink-receiving layer of not less than 1.5.

**23 Claims, 2 Drawing Sheets**



FOREIGN PATENT DOCUMENTS

|    |              |         |
|----|--------------|---------|
| EP | 0 634 287 A1 | 1/1995  |
| JP | 54-59936     | 5/1979  |
| JP | 56-76246     | 6/1981  |
| JP | 56-95985     | 8/1981  |
| JP | 2-276670     | 11/1990 |
| JP | 4-37576      | 2/1992  |
| JP | 5-32037      | 2/1993  |

OTHER PUBLICATIONS

The Journal of the American Chemical Society vol. LX, dated Jan.-Jun. 1938, pp. 309-319.

R. Tettenhorst, et al., "Crystal Chemistry of Boehmite", Clays and Clay Minerals, vol. 28, No. 5, pp. 373-380, 1980.

\* cited by examiner

FIG. 1



FIG. 2A



FIG. 2B



FIG. 2C



PLANE DIRECTION OF  
THE INK-RECEIVING LAYER

FIG. 2D



FIG. 3A



FIG. 3B



## 1

**RECORDING MEDIUM, PROCESS FOR  
PRODUCTION THEREOF, AND INK-JET  
RECORDING METHOD EMPLOYING THE  
MEDIUM**

This application is a continuation of application Ser. No. 08/528,208 filed Sep. 12, 1995, now abandoned.

**BACKGROUND OF THE INVENTION**

**1. Field of the Invention**

The present invention relates to a recording medium suitable for recording with aqueous ink, particularly to a recording medium suitable for ink-jet recording.

**2. Related Background Art**

Ink-jet recording is a method for recording images and letters by ejecting fine droplets of ink onto a recording medium such as a paper sheet. Ink-jet recording is rapidly becoming popular in recent years for various applications because of its high recording speed, ease of multicolor recording, flexibility in pattern recording, and because image fixation is not needed. Multicolor ink-jet recording is coming to be used in full color image recording since it is capable of giving images comparable with images formed by multicolor gravure printing or color photography, and is less expensive than multicolor printing when the number of reproduction is small. With improvements in recording speed, fineness of recording, and full color recording, the recording medium is required to have better qualities in addition to the improvements of the recording apparatus and the recording method.

Hitherto, various types of recording mediums have been disclosed. For example, recording sheets having a layer containing alumina hydrate of pseudo boehmite structure are disclosed in U.S. Pat. Nos. 4,879,166 and 5,104,730, and Japanese Patent Laid-Open Application Nos. 2-276670, 4-37576, and 5-32037. The prior art recording mediums involve disadvantages as follows: occurrence of beading of ink dots, due to insufficient absorbency for a large amount of ink in color image printing; likelihood of being scratched by sheet delivery device due to insufficient surface hardness; likelihood of the ink-receiving layer surface cracking due to insufficient bonding strength of the ink-receiving layer; low circularity of printed dots due to insufficient uniformity of the ink-receiving layer; and low gloss of recording medium due to less orientation of the pigment.

The beading mentioned in the present invention refers to a phenomenon in which dots irregularly move in the plane direction of the surface of an ink-receiving layer when the ink is still fluid before it is fixed in the ink-receiving layer.

The present invention has been made to offset the above disadvantages.

**SUMMARY OF THE INVENTION**

An object of the present invention is to provide a recording medium which has high ink absorbency to absorb ink at a higher absorbing rate and having higher surface hardness to be less liable to cracking on the surface.

Another object of the present invention is to provide a recording medium which is capable of forming an image with high circularity of dots and high gloss of the recorded image.

Still another object of the present invention is to provide a recording medium which provides water fastness and light fastness of the recorded image with less migration of the ink, in addition to the aforementioned properties.

## 2

A further object of the present invention is to provide a process for producing the aforementioned recording medium.

5 A still further object of the present invention is to provide an ink-jet recording method employing the aforementioned recording medium.

According to an aspect of the present invention, there is provided a recording medium having a porous ink-receiving layer containing alumina hydrate of boehmite structure formed on a base material, the alumina hydrate having crystallinity ranging from 15 to 80.

10 According to another aspect of the present invention, there is provided a recording medium having a porous ink-receiving layer containing alumina hydrate of boehmite structure formed on a base material, wherein microcrystals of the alumina hydrate are directed to be parallel to the plane direction of the ink-receiving layer at a parallelization degree of not less than 1.5.

15 According to still another aspect of the present invention, there is provided a recording medium having a porous ink-receiving layer containing alumina hydrate of boehmite structure formed on a base material, the alumina hydrate having crystallinity ranging from 15 to 80, and the microcrystals of the alumina hydrate being directed to be parallel to the plane direction of the ink-receiving layer at a parallelization degree of not less than 1.5.

20 According to a further aspect of the present invention, there is provided an ink-jet recording method employing the above recording medium.

25 According to a still further aspect of the present invention, there is provided a process for producing a recording medium having a porous ink-receiving layer containing alumina hydrate of boehmite structure, comprising the steps of: applying a coating liquid containing alumina hydrate of boehmite structure with shearing stress onto a base material; and drying the coated material to obtain the degree of 30 parallelization of the microcrystal of the alumina hydrate with the plane direction of the ink-receiving layer of not less than 1.5.

35 According to a still further aspect of the present invention, there is provided a process for producing a recording medium, comprising the steps of: applying a liquid dispersion containing alumina hydrate of boehmite structure having crystallinity ranging from 15 to 80 onto a base material; and drying the coated material at a relative humidity of 20 to 40 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615

## BRIEF DESCRIPTION OF THE PREFERRED EMBODIMENTS

FIG. 1 is a schematic sectional view for explaining a recording medium of the present invention.

FIGS. 2A to 2D are schematic sectional views for explaining the degree of parallelization of the microcrystals in the recording medium of the present invention.

FIGS. 3A and 3B are schematic sectional views for explaining the dependency of ink absorbing rate on the direction of the planes (020) of microcrystalline alumina hydrate in the recording medium of the present invention.

## DESCRIPTION OF PREFERRED EMBODIMENTS

The recording medium according to the present invention exhibits high ink absorbency, absorbs ink at a high rate, has sufficient surface hardness, is less liable to cause cracking of the surface, provides high circularity of printed dots, and has high gloss. The recording medium gives high water fastness and high light-fastness to the recorded matter with less migration of the recording liquid.

The recording medium of the present invention, in an embodiment, has one ink-receiving layer 2 of a porous structure comprising alumina hydrate and a binder provided on a base material 1.

The alumina hydrate, which is positively charged, is preferred as the constituting material for the ink-receiving layer, since it fixes the applied ink by a positive charge to give excellent colors to images, and does not involve the disadvantages of browning of black ink and low light-fastness which are problems associated with the use of a silica type compound for the ink-receiving layer. Of the alumina hydrates, one having boehmite structure is more suitable because of high adsorbability of dyes, high absorbency of ink, and high transparency.

The alumina hydrate contained in the recording medium of the present invention is defined by the general formula below:



where n is an integer of zero to 3, and m is a number of from zero to 10, preferably from zero to 5. In many cases, "mH<sub>2</sub>O" expresses a free water phase which does not contribute to the construction of a crystal lattice and is releasable. Therefore, the value of "m" is not necessarily an integer. The value of "m" may become zero when the alumina is calcined.

The process for producing the alumina hydrate having a boehmite structure to be incorporated into the recording medium of the present invention is not specially limited. The process includes Bayer process, alum pyrolysis process, and other processes for producing alumina hydrate. A suitable process is hydrolysis of a long-chain alkoxide of aluminum by addition of an acid. The long-chain alkoxide herein means alkoxides of 5 or more carbons, more preferably alkoxides of 12 to 22 carbons. With such an aluminum alkoxide, removal of the alcohol component and control of the shape of the alumina hydrate of boehmite structure are facilitated. The above-mentioned processes are advantageous because of less likelihood of contamination by ions and other impurities in comparison with processes using alumina hydrogel or cationic alumina. Further, long-chain alkoxides of aluminum are advantageous in that the alcohol resulting from the hydrolysis can readily be removed com-

pletely from the alumina hydrate in comparison with short-chain alkoxides such as aluminum isopropoxide.

The alumina hydrate prepared by the above process may be subjected to hydrothermal synthesis to allow the particles to grow, or may be dried to obtain powdery alumina hydrate.

In the present invention, a liquid dispersion containing the alumina hydrate and a binder is applied onto a base material, and the applied matter is subjected to drying and other treatments to form a recording medium having a porous ink-receiving layer. The properties of the recording medium depend on the alumina hydrate employed, the liquid dispersion, and the conditions of production such as coating application and drying. In the present invention, it was found that the ink absorbency of the porous ink-receiving layer can be improved and the cracking thereof can be prevented by control of the crystallinity and the parallelization degree of the alumina hydrate in the layer.

The crystallinity in the present invention is defined as follows:

As shown in FIG. 2A, particles of alumina hydrate 6 having boehmite structure contained in the ink-receiving layer 2 are constituted of non-crystalline portions 10 and crystalline portions (boehmite microcrystals) 3.

The crystallinity degree means the ratio of crystalline portion to the entire alumina hydrate having a boehmite structure.

The crystallinity is derived from an X-ray diffraction pattern measured by CuK $\alpha$  line of the pulverized ink-receiving layer, from the ratio of the peak intensity of the plane (020) appearing at about 20=14°-15° to the peak intensity at 20=10°. The crystallinity is disclosed in Japanese Patent Laid-Open Application Nos. 56-76246 and 56-95985.

In the present invention, the crystallinity of the alumina hydrate in the ink-receiving layer is preferably in the range of from 15 to 80. Within this range, the ink absorbency and the ink absorbing rate are satisfactory. More preferably, the crystallinity ranges from 20 to 70. Within this range, the surface hardness is higher, and the cracking is less likely to occur. At a crystallinity lower than 15, the ink absorbency and the ink absorbing rate are insufficient, whereas at a crystallinity higher than 80, the affinity to water is lower, which makes beading of ink dots likely to occur.

The parallelization degree in the present invention is defined as follows. As shown in FIG. 2A, the parallelization degree relates to the ratio of fine boehmite crystals 3 having (020) planes parallel to the plane direction of the ink-receiving layer to the entire fine boehmite crystals contained in the ink-receiving layer. FIG. 2D shows the plane direction of alumina hydrate fine crystals drawn in FIGS. 2A, 2B and 2C. The alumina hydrate has planes (020) 4 and planes (120) 5 as shown in FIG. 2D.

To measure the parallelization degree, the ratio of the intensities of X-ray diffraction peaks measured by CuK $\alpha$  line of plane (020) to that of plane (120) is derived for the ink-receiving layer (Ratio A); and separately the same ratio is derived for the pulverized ink-receiving layer (Ratio B). The parallelization degree is represented by the ratio of Ratio A to Ratio B.

When the planes (020) are directed completely at random, the parallelization degree of the ink-receiving layer is 1. As shown in FIGS. 2A to 2C, a higher parallelization degree means a higher ratio of the plane (020) parallel to the ink-receiving layer face. The parallelization degrees in FIGS. 2A, 2B and 2C are low, moderate, and high, respectively.

The recording medium of the present invention has a parallelization degree of preferably not less than 1.5 to obtain a higher circularity of the printed dots. If the parallelization degree is less than 1.5, the circularity of the printed dots is low. The parallelization degree is more preferably 2 or higher, thereby making the gloss of the recording medium higher.

The mechanism of ink absorption in the recording medium of the present invention is assumed to be as described below. The ink droplets deposited on the surface of the recording medium are absorbed mainly by the interspaces between the planes (020) in the alumina hydrate particles. In a recording medium having a low parallelization degree as shown in FIG. 3A, the deposited ink diffuses non-uniformly, due to random orientation of the crystal planes (020) in the ink-receiving layer face direction. On the other hand, in a recording medium having a high parallelization degree as shown in FIG. 3B, the ink diffuses uniformly in the recording layer face direction. Thereby, the circularity of the printed dots is presumed to be higher in the recording medium having the parallelization degree of 1.5 or more. In FIGS. 3A and 3B, the numeral 7 indicates a microcrystal of alumina hydrate particle into which ink 8 has penetrated. The numeral 9 indicates a printing head of the printer.

The light refractivity of the alumina hydrate at the crystalline portion differs from that at the non-crystalline portion. Therefore, the recording medium having randomly oriented crystal plane (020) of the alumina hydrate exhibits more noticeable light scattering than one having uniformly oriented planes (020). Therefore, a recording medium having a parallelization degree of 2 or higher exhibits lower light scattering and has higher gloss, presumably.

The recording medium, which has crystallinity of the alumina hydrate of from 15 to 80 and a parallelization degree of the alumina hydrate microcrystal of 1.5 or higher, has high water resistance and high light-fastness, and does not cause migration of the dye during storage, desirably. When the crystallinity is outside the above range, the affinity of the recording medium to the ink is lower, which causes migration repulsion, and beading of the ink, and retards the ink absorption. With the parallelization degree outside the above range, migration of the ink is likely to occur, due to the lower bonding strength of the dye to the recording medium. The dye of the ink, is adsorbed by the interspaces between the crystal planes (020) of alumina hydrate microcrystals. The adsorbed dye is less releasable in the recording medium having higher parallelization degree due to higher adsorption strength caused by interaction of the uniformly orientated alumina crystal planes (020). This is because the recording medium having a higher parallelization degree has a lot of alumina microcrystal planes (020), whereby many adsorbing points are provided therein, and if the recording medium has a higher parallelization degree too, the planes (020) are uniformly oriented. Therefore, the above-mentioned effects can be obtained with the recording medium having the crystallinity and parallelization degree in the aforementioned ranges.

The aforementioned Japanese Patent Laid-Open Application No. 2-276670 describes a recording medium employing an agglomerate of fine alumina particle oriented in one direction which is formed by orienting particles of alumina hydrate, and has a constitution different from the recording medium having a specified parallelization degree of the planes (020) of the present invention. Furthermore, this Japanese Patent Laid-Open Application does not mention

the circularity and the gloss which are the effects of the present invention, and is based on an idea different from the present invention.

The crystallinity of the alumina hydrate in the recording medium can be changed by controlling the heating conditions in drying the alumina hydrate-containing dispersion, and the parallelization degree can independently be changed by shearing stress on application of the dispersion.

The crystallinity of the alumina hydrate employed in the present invention is preferably in the range of from 15 to 80, since crystallinity within this range can be attained easily. The alumina hydrate which has a crystallinity of less than 15 can be changed to have higher crystallinity in later processing. The alumina hydrate may be in a needle shape or in a plate shape. The particle size of the alumina hydrate is preferably in the range of from 1 to 50 nm in the maximum length for a needle-shaped particle or in the maximum diameter for a plate-shaped particle, since the viscosity of the dispersion is low and cracking or powder-falling is less likely to occur in this particle size range. The alumina hydrate has preferably a pore volume ranging from 0.1 to 1.0 cm<sup>3</sup>/g, and a pore radius ranging from 2.0 to 20.0 nm in view of ink absorbency. The specific surface area of the alumina hydrate ranges preferably from 10 to 500 m<sup>2</sup>/g in view of the low haze of the ink receiving layer for obtaining a glossy image and for observing an image by transmitted light.

The recording medium of the present invention can be prepared by applying a liquid dispersion containing the alumina hydrate and a binder onto a base material. By controlling the shearing stress in a specified range on application of the liquid dispersion onto the base material, the microcrystal planes (020) can be oriented in the direction parallel to the flow of the coating liquid dispersion, whereby the recording medium is made to have a high parallelization degree. The required shearing stress depends on the coating method and the viscosity of the liquid dispersion, and ranges preferably from 0.1 to 20.0 N/m<sup>2</sup>. In this range of shearing stress, microcrystals of the alumina hydrate are oriented to have a parallelization degree of 1.5 or more. When the shearing stress is lower than the above range, it is difficult to make the parallelization degree 1.5 or higher. With the shearing stress higher than the above range, the resulting ink-receiving layer tends to be non-uniform in thickness.

The coating may be conducted by any method, provided that the shearing stress in the above range can be applied. The preferred coating method includes kiss-roll coating, extrusion coating, slide hopper coating, curtain coating, blade coating, brush coating, bar coating, and gravure coating.

The suitable coating speed depends on the coating method. With a coating method in which the shearing stress depends on the coating speed, such as kiss-roll coating, extrusion coating, slide hopper coating, curtain coating, and bar coating, the coating speed ranges preferably from 0.01 to 10 m/s. At a coating speed of lower than 0.01 m/s, little shearing stress will be applied, and the parallelization degree tends to be lower. At a coating speed of higher than 10 m/s, the thickness of the ink-receiving layer is not readily controllable uniformly. The viscosity of the liquid dispersion at the time of the coating ranges preferably from 10 to 500 mPa·s. At the viscosity of lower than 10 mPa·s, the shearing stress given to the liquid dispersion is lower, and thereby the parallelization degree of alumina hydrate microcrystals in the resulting recording medium tends to be lower. At a viscosity of higher than 500 mPa·s, the thickness of the ink-receiving layer is not readily controllable uniformly. The

amount of the coating of the liquid dispersion ranges preferably from 2 to 60 g/m<sup>2</sup> in terms of the dried solid matter.

The liquid dispersion after coating application is dried preferably without blowing of drying air thereon, at least for one second to be thickened and set in an oriented state of the microcrystal planes (020) of the alumina hydrate by utilizing thixotropy of the liquid dispersion. If drying air is blown on the unset coating layer, it displaces the particles of the alumina hydrate destroys the oriented state of the crystal planes (020) of the alumina hydrate, which were made by the shearing stress, resulting in a low parallelization degree.

The applied coating liquid dispersion containing the alumina hydrate forms the ink-receiving layer by heat-drying. It was found that the crystallinity can be controlled to be within the above specified range by controlling the heating rate, drying temperature, and drying time. Particularly, the crystallinity depends on the drying speed.

Therefore, the crystallinity can be controlled within the above range by controlling the humidity, temperature and drying time in the process of drying the liquid dispersion. When the recording medium is prepared from alumina hydrate having a crystallization degree of from 15 to 80 dispersed in a coating liquid dispersion, drying at a relative humidity ranging from 20% to 60% gives the alumina hydrate in the resulting recording medium a crystallinity in the above specified range. Drying at a relative humidity lower than 20% makes it difficult to control the crystallinity of the recording medium because of the large change in the crystallinity of the alumina hydrate per unit time. Drying at a relative humidity higher than 60% tends to cause non-uniform thickness of the ink-receiving layer because of the lower drying speed of the coating film.

When the recording medium is prepared from alumina hydrate having crystallization degree of lower than 15 dispersed in a coating liquid dispersion, drying at the relative humidity ranging from 10% to 20% gives the crystallinity of the alumina hydrate in the resulting recording medium in the above specified range. Further, an alternative process can be provided, which comprises applying onto a base material a liquid dispersion containing alumina hydrate having a crystallinity of lower than 15, followed by drying the liquid dispersion to form an ink receiving layer, and heating the obtained recording medium at a relative humidity of 10 to 20%, whereby it is possible to control the crystallinity within the above-mentioned range. Drying at a relative humidity lower than 10% makes it difficult to control the crystallinity to be not higher than 80 because of the rapid rise in the crystallinity of the alumina hydrate per unit time. In this case, it is also likely to generate cracking. Drying at a relative humidity of higher than 20% does not result in the intended crystallinity because of lack of increase in of the crystallinity.

The most suitable heat-drying conditions (temperature and time) depend on the composition of the coating liquid, but are generally a heating temperature ranging from 60° C. to 150° C., and a heating time ranging from 2 seconds to 30 minutes. It is difficult to achieve the crystallinity in the above specified range at a drying temperature of lower than 60° C. even at the aforementioned humidity range. At a drying temperature higher than 150° C., the crystallinity will exceed the above specified range due to excessively high drying speed, and furthermore the ink-receiving layer is likely to be cracked. At a drying time of less than 2 seconds, the formed ink-receiving layer will become non-uniform in layer thickness because of insufficient drying time. A drying

time of longer than 30 minutes is not effective since the change of the crystallinity will be finished within 30 minutes.

The above heating process can be conducted with a drying apparatus including hot air driers such as a direct tunnel drier, an arch drier, an air loop drier, and a sine-curve air float drier; infrared heating driers; microwave driers; and heating rolls.

The binder which may be used with the alumina hydrate in the present invention may be selected from water-soluble polymers, including preferably polyvinyl alcohol and modifications thereof (cation-modified, anion-modified, and silanol-modified), starch and modifications thereof (oxidized, and etherified), gelatin and modifications thereof, casein and modifications thereof, gum arabic, cellulose derivatives such as carboxymethylcellulose, hydroxyethylcellulose, and hydroxypropylmethylcellulose, SBR latexes, NBR latexes, diene type copolymer latex such as methyl methacrylate-butadiene copolymer latex, functional group-modified polymer latexes, vinyl copolymer latexes such as ethylene-vinyl acetate copolymer latex, polyvinylpyrrolidones, maleic anhydride copolymers, acrylic ester copolymers, and the like.

The mixing weight ratio of the alumina hydrate having boehmite structure to the binder ranges preferably from 5:1 to 25:1. Within this range, the cracking or the powder-falling of the ink-receiving layer can be prevented. The mixing weight ratio ranges more preferably from 5:1 to 20:1. Within this range, cracking can be prevented which is caused by folding of the recording medium.

To the pigment and the binder, there may be added a pigment dispersant, a viscosity increaser, a pH controller, a lubricator, a fluidity modifier, a surfactant, an antifoaming agent, water-proofing agent, a foam inhibitor, a releasing agent, a foaming agent, a penetrating agent, a coloring dye, a fluorescent whitener, an ultraviolet absorber, an antioxidant, an antiseptic agent, a mildewproofing agent, and the like. The water-proofing agent may be selected from known materials such as quaternary ammonium salts, and polymeric quaternary ammonium salts.

The base material may be a paper sheet such as a sized paper sheet, a non-sized paper sheet, or a resin-coated paper; a sheet-shaped material such as a thermoplastic resin film; or cloth. The thermoplastic resin film may be a transparent film of a resin such as polyester, polystyrene, polyvinyl chloride, polymethyl methacrylate, cellulose acetate, polyethylene, or polycarbonate; or a pigment-filled or finely-foamed opaque plastic sheet.

The ink-receiving layer constituting the recording medium of the present invention has a total pore volume ranging preferably from 0.1 to 1.0 cm<sup>3</sup>/g. With a pore volume larger than the above range, the ink-receiving layer is likely to cause cracking or powder-falling therefrom. With the pore volume smaller than the above range, the ink-receiving layer exhibits low ink-absorbency, and is likely to cause migration of ink on the ink-receiving layer particularly in multicolor printing.

The ink-receiving layer has a BET specific surface area preferably ranging from 20 to 450 m<sup>2</sup>/g. With a specific surface area smaller than this range, the ink-receiving layer is not glossy, and has a high haze which gives a hazed image. With a specific surface area larger than the above range, the ink-receiving layer is likely to crack. The aforementioned BET specific surface area and the pore volume are measured, after degassing treatment at 120° C. for 24 hours, by a nitrogen adsorption-desorption method.

The ink employed in the recording according to the present invention comprises a coloring material (dye or pigment), a water-soluble organic solvent, and water as the main constituents. The dye is preferably a water-soluble dye such as a direct dye, acid dye, basic dye, reactive dye, or food dye. Any dye may be used, provided that it has the required properties such as fixability, color-developability, sharp image formation, stability, and light-fastness in combination with the recording medium.

The water-soluble dye is generally used as a solution in water or a mixed solvent of water and an organic solvent. The solvent is preferably a mixture of water and a water-soluble organic solvent. The water content in the ink ranges preferably from 20% to 90%, more preferably from 60% to 90% by weight.

The aforementioned water soluble organic solvent includes alkyl alcohols of 1 to 4 carbons such as methyl alcohol, ethyl alcohol, n-propyl alcohol, isopropyl alcohol, n-butyl alcohol, s-butyl alcohol, t-butyl alcohol, and isobutyl alcohol; amides such as dimethylformamide, and dimethylacetamide; ketones and ketone alcohols such as acetone, and diacetone alcohol; ethers such as tetrahydrofuran, and dioxane; polyalkylene glycols such as polyethylene glycol, and polypropylene glycol; alkylene glycols having an alkylene group of 2 to 6 carbons such as ethylene glycol, propylene glycol, 1,2,6-hexanetriol, thiadiglycol, hexylene glycol, and diethylene glycol; glycerol; lower alkyl ethers of polyhydric alcohols such as ethylene glycol methyl ether, diethylene glycol monomethyl ether, diethylene glycol ethyl ether, triethylene glycol monomethyl ether, and triethylene glycol monoethyl ether; and the like.

Of these water-soluble organic solvents, polyhydric alcohols such as diethylene glycol, and lower alkyl ethers of polyhydric alcohols such as triethylene glycol monomethyl ether, and triethylene glycol monoethyl ether are preferred. The polyhydric alcohols are advantageous since they serve as a lubricant for preventing the clogging of nozzles caused by deposition of the water-soluble dye resulting from evaporation of water from the ink.

The ink may contain a solubilizing agent, typically a nitrogen-containing heterocyclic ketone, for increasing remarkably the solubility of the water-soluble dye in the solvent. The examples of the effective solubilizing agent are N-methyl-2-pyrrolidone, and 1,3-dimethyl-2-imidazolidinone. For further improvement of the properties, there may be added an additive such as a viscosity improver, a surfactant, a surface tension controller, a pH controller, a specific resistance improver, and the like.

On the recording medium, recording is conducted with the above ink preferably by ink-jet recording. Any ink-jet recording method is applicable which ejects ink through a nozzle to deposit the ink on the recording medium. In particular, the method disclosed in Japanese Patent Laid-Open Application No. 54-59936 is effective. In this method, thermal energy is applied to the ink to cause an abrupt volume change of the ink to eject the ink through the nozzle by the action of the volume change.

The present invention is described in more detail by reference to Examples and Comparative Examples. The properties of the present invention were measured by the procedures below.

#### [Crystallinity and Parallelization Degree]

The ink-receiving layer was separated from the recording medium, pulverized, and subjected to X-ray diffraction measurement. The diffraction intensity was measured at  $2\theta=10^\circ$ , and the diffraction peak intensities were measured

for the plane (020) and the plane (120), from the X-ray diffraction pattern. Independently, the diffraction peak intensities of the separated ink-receiving layer, not pulverized, were measured similarly for the plane (020) and the plane (120) from the X-ray diffraction pattern. The crystallinity and the parallelization degree were derived according to the equations below.

$$\text{Crystallinity} = \frac{\text{Peak intensity for plane (020)}}{\text{intensity at } 2\theta = 10^\circ}$$

$$\text{Intensity ratio for powder} = \frac{\text{Peak intensity for plane (020) of powder}}{\text{Peak intensity for plane (120) of powder}}$$

$$\text{Intensity ratio for medium} = \frac{\text{Peak intensity for plane (020) of medium}}{\text{Peak intensity for plane (120) of medium}}$$

(Ink-receiving layer)

$$\text{Parallelization degree} = \frac{\text{Intensity ratio for medium}}{\text{Intensity ratio for powder}}$$

The conditions for the above X-ray diffraction measurement were as below:

|                 |                                                                                                          |
|-----------------|----------------------------------------------------------------------------------------------------------|
| Apparatus:      | RAD-2R (Rigaku Denki K.K.)                                                                               |
| Target:         | CuK $\alpha$                                                                                             |
| Optical system: | Wide angle goniometer<br>(with curved graphite monochromator)                                            |
| Gonio radius:   | 185 mm                                                                                                   |
| Slits:          | DS 1°, RS 1°, SS 0.15 mm                                                                                 |
| X-ray output:   | 40 kV, 30 mA                                                                                             |
| Measurement:    | Method of 20-0<br>Continuous scanning, every 0.02° for 20<br>$2\theta = 10^\circ$ to $90^\circ$ , 2°/min |

#### [BET Specific Surface Area, and Pore Volume]

The specific surface area and the pore volume were measured, after sufficient heating and degassing treatment of the recording medium, by the nitrogen adsorption-desorption method.

#### Measurement apparatus: Autosorb 1 (Quanta Chrome Co.)

The BET specific surface area was calculated according to the method of Brunauer, et al. (J. Am. Chem. Soc., Vol.60, p.309, (1938)).

The pore volume was calculated according to the method of Barrett, et al. (J. Am. Chem. Soc., Vol.73, p.373 (1951)).

#### [Ink Absorbency]

Ink-jet recording was conducted by an ink-jet printer provided with an ink-jet head having 128 nozzles for four colors of Y, M, C, and Bk with the nozzle spacing of 16 nozzles per mm by use of the inks having the compositions shown below. The ink absorbency was evaluated by solid-printing singly with a Bk color ink and immediately thereafter testing the ink drying state at the surface of the ink-receiving layer by finger touch. The usual amount of ink for single color printing was prescribed to be 100%. The ink absorbency of the recording medium was evaluated to be "good" when the ink did not transfer to the finger with the amount of the ink of 200%; to be "fair" when the ink did not transfer to the finger with the amount of 100%; and to be "poor" when the ink transferred to the finger with the amount of 100%.

Ink Composition:

|                     |          |
|---------------------|----------|
| C.I. Food Black 2   | 5 parts  |
| Diethylene glycol   | 15 parts |
| Polyethylene glycol | 20 parts |
| Water               | 70 parts |

[Ink Absorption Rate]

Bk single color solid printing was conducted with the same ink-jet printer and the same ink as the ones used in the above ink absorbency test with an amount of ink of 200%. The drying state was tested by finger touch on the printed area, and the time elapsed before the ink became non-transferable to the touching finger was measured.

[Surface Hardness]

The surface hardness was tested according to the pencil scratch test for paint film of JIS K5401-1969.

[Cracking]

Occurrence of cracking at the surface of the recording medium was examined visually. The recording medium was evaluated to be "good" when no cracking was observed; to be "fair" when cracking was observed locally; and to be "poor" when cracking occurs over the entire surface.

[Circularity]

Bk printing was conducted dot by dot by using the same ink jet printer and the same ink as the ones used in the above ink absorbency test. The major diameter D and the minor diameter d of one dot was measured by microscopy. The ratio of d/D was taken as the measure of the circularity.

[Gloss]

The gloss of the recording medium at the non-printed area was measured by a gloss meter (Gloss Checker-IG-320, Horiba Seisakusho K.K.).

[Water fastness]

Single color solid-printing was conducted by using the same ink jet printer and the same ink as the ones used in the above ink absorbency test. The printed recording medium was immersed in flowing water for 3 minutes, and was air-dried. The water-resistance was represented by the equation below.

$$\text{Water resistance} = \frac{\text{Image density after water immersion}}{\text{Image density before water immersion}} \times 100$$

The recording medium was evaluated to be "good" when the water resistance was higher than 95, to be "fair" when the resistance was in the range of from 88 to 95, and to be "poor" when the resistance was lower than 88.

[Light-fastness]

Bk single color solid-printing was conducted with the same ink-jet printer and the same ink in the above ink absorbency test. The ink was used in an amount of 100%. Thereafter, the printed recording medium was left standing at room temperature. The color tone (L\*) of the printed area was measured one day and 30 days after the printing, and the change ratio was derived. The recording medium was evaluated to be "good" when the change ratio was not more than  $\pm 10\%$ , to be "fair" when it was not more than  $\pm 20\%$ , and to be "poor" when it was more than  $\pm 20\%$ .

[Migration]

One-dot printing of single color was conducted with the same ink-jet printer and the same ink as the ones used in the above ink absorbency test. The major diameters of the ink dots were measured one day and 30 days after the printing. The migration of the ink is prescribed by the equation below:

$$10 \quad \text{Migration} = \frac{\text{Major diameter after 30 days}}{\text{Major diameter after one day}} \times 100$$

15 The recording medium was evaluated to be "good" in view of absence of migration of ink when the above value of migration was less than 105, to be "fair" when it was in the range of from 105 to 110, and to be "poor" when it was more than 110.

20 EXAMPLES 1 to 4

25 Aluminum dodecyloxide was prepared according to by weight to obtain an alumina liquid dispersion. Separately, polyvinyl alcohol (trade name: Gosenol NH18 (hereinafter referred to as "PVA"), Nippon Gosei Kagaku K.K.) was mixed with deionized water at a concentration of 17% by weight to obtain a PVA solution. The alumina liquid dispersion and the PVA solution were mixed at a mixing ratio of 18:1 to obtain a coating liquid. This coating liquid was 30 applied onto a resin-coated paper sheet by means of an extrusion coater at a coating temperature of 100° C. under shearing stress of 7.5 N/m<sup>2</sup> (75 dyn/cm<sup>2</sup>), and was delivered without blowing of drying air for one second to thicken and set the coating layer by utilizing thixotropy. Then the coating 35 layer was dried for 30 seconds in an environment of relative humidity of 40% at a temperature shown in Table 2. The resulting recording medium was evaluated for the printing properties, etc. The evaluation results are shown in Table 2. the method described in U.S. Pat. No. 4,242,271. Then the 40 resulting aluminum dodecyloxide was hydrolyzed into alumina in a slurry state according to the method described in U.S. Pat. No. 4,202,870. To this alumina slurry, water was added to dilute it to the content of solid alumina hydrate of boehmite structure of 7.9% in the slurry. The alumina slurry 45 showed a pH of 9.5. The pH was adjusted by adding 3.9% nitric acid solution. The slurry was aged under the conditions shown in Table 1 to obtain colloidal sols. This colloidal sols were spray-dried at 85° C. to obtain samples of powdery alumina hydrate of boehmite structure.

50

TABLE 1

| 55                                            | Aging Condions of Alumina hydrate |      |      |      |
|-----------------------------------------------|-----------------------------------|------|------|------|
|                                               | Example No.                       |      |      |      |
|                                               | 1                                 | 2    | 3    | 4    |
| pH before aging                               | 6.6                               | 6.6  | 6.8  | 6.4  |
| Aging temperature (° C.)                      | 48                                | 49   | 50   | 35   |
| Aging period (days)                           | 14                                | 16   | 18   | 16   |
| Aging apparatus                               | Oven                              | Oven | Oven | Oven |
| Crystallinity                                 | 20.2                              | 31.0 | 45.5 | 26.1 |
| BET specific surface area (m <sup>2</sup> /g) | 200                               | 180  | 210  | 230  |
| Pore volume (cm <sup>3</sup> /g)              | 0.70                              | 0.75 | 0.71 | 0.68 |

65 The alumina hydrate of boehmite structure was dispersed in deionized water at a concentration of 17%

TABLE 2

|                                               | Evaluation results |      |      |      |
|-----------------------------------------------|--------------------|------|------|------|
|                                               | Example No.        |      |      |      |
|                                               | 1                  | 2    | 3    | 4    |
| Drying temperature (° C.)                     | 72                 | 80   | 90   | 72   |
| Crystallinity                                 | 19.8               | 32.2 | 47.5 | 28.1 |
| BET specific surface area (m <sup>2</sup> /g) | 180                | 165  | 185  | 195  |
| Pore volume (cm <sup>3</sup> /g)              | 0.50               | 0.58 | 0.56 | 0.51 |
| Ink Absorbency                                | Good               | Good | Good | Good |
| Ink absorption rate (seconds)                 | <10                | <10  | <10  | <10  |
| Surface hardness                              | HB                 | H    | H    | H    |
| Cracking                                      | Fair               | Good | Good | Good |

## EXAMPLE 5

A recording medium (before heating) was prepared in the same manner as in Examples 1 to 4 except that the aging conditions and drying conditions of the alumina hydrate were changed as shown in Table 3, the drying temperature was 68° C., the drying time was 30 seconds and the relative humidity was 50%. The resulting recording medium was further heated for 30 minutes in an oven kept at a temperature of 80° C. and a relative humidity of 12% (recording medium after heating). The properties of the recording medium before and after heating are shown in Table 4. The heating treatment of the recording medium in this Example increases the crystallinity thereof, and thereby improving the ink absorbency, as shown in Table 4.

TABLE 3

Aging conditions of Alumina hydrate in Examples 5, and 6-11

|                                               | Example No. |      |      |
|-----------------------------------------------|-------------|------|------|
|                                               | 5           | 6-10 | 11   |
| pH before aging                               | 6.4         | 6.3  | 6.1  |
| Aging temperature (° C.)                      | 32          | 34   | 33   |
| Aging period (days)                           | 15          | 18   | 16   |
| Aging apparatus                               | Oven        | Oven | Oven |
| Crystallinity                                 | 10.0        | 47.2 | 12.0 |
| BET specific surface area (m <sup>2</sup> /g) | 220         | 235  | 230  |
| Pore volume (cm <sup>3</sup> /g)              | 0.73        | 0.75 | 0.71 |

TABLE 4

Evaluation Results in Example 5

|                                               | Before heating | After heating |
|-----------------------------------------------|----------------|---------------|
| Crystallinity                                 | 10.0           | 19.0          |
| Parallelization degree                        | 2.2            | 2.2           |
| BET specific surface area (m <sup>2</sup> /g) | 190            | 190           |
| Pore volume (cm <sup>3</sup> /g)              | 0.56           | 0.56          |
| Ink Absorbency                                | Fair           | Good          |
| Ink absorption rate (seconds)                 | 17             | <10           |
| Surface hardness                              | F              | H             |
| Cracking                                      | Fair           | Good          |
| Circularity                                   | 0.89           | 0.87          |
| Gloss                                         | 52             | 53            |

## EXAMPLES 6 to 10

5 Alumina hydrate liquid dispersions were prepared in the same manner as in Examples 1-4 except that the aging conditions and drying conditions were changed as shown in Table 3. The liquid dispersion was applied by means of an extrusion coater and dried. The shearing stress given to the coating liquid was adjusted to be 0.2 N/m<sup>2</sup> (Example 6), 6.0 N/m<sup>2</sup> (Example 7), 10.0 N/m<sup>2</sup> (Example 8), 14.0 N/m<sup>2</sup> (Example 9), and 18.0 N/m<sup>2</sup> (Example 10) respectively by changing the slit width and the extrusion pressure. The amount of the coating was 6 g/m<sup>2</sup> in each Example.

10 The coating was conducted at a rate of 1 m/s. The coated material was delivered without blowing of drying air for one second after the coating application to thicken and set the coating by utilizing thixotropy of the coating liquid, and then it was dried for 20 seconds at 90° C. at a relative humidity of 40%.

15 The resulting recording mediums were evaluated for printing properties. The results are shown in Table 5. The recording mediums prepared in these Examples changed their parallelization degree depending on the shearing stress given to the coating liquid, thereby changing the gloss.

TABLE 5

|                                               | Evaluation Results in Examples 6-10 |      |      |      |      |
|-----------------------------------------------|-------------------------------------|------|------|------|------|
|                                               | Example No.                         |      |      |      |      |
|                                               | 6                                   | 7    | 8    | 9    | 10   |
| Shearing stress (N/m <sup>2</sup> )           | 0.2                                 | 6.0  | 10.0 | 14.0 | 18.0 |
| Parallelization degree                        | 2.2                                 | 3.3  | 3.5  | 3.1  | 2.1  |
| BET specific surface area (m <sup>2</sup> /g) | 193                                 | 193  | 193  | 193  | 193  |
| Pore volume (cm <sup>3</sup> /g)              | 0.57                                | 0.57 | 0.57 | 0.57 | 0.57 |
| Circularity                                   | 0.88                                | 0.92 | 0.95 | 0.93 | 0.87 |
| Gloss                                         | 53                                  | 62   | 68   | 59   | 51   |

## EXAMPLE 11

45 Alumina hydrate liquid dispersion was prepared in the same manner as in Example 1 except that the aging conditions and the drying conditions were changed as shown in Table 3. With this liquid dispersion, a recording medium was prepared in the same manner as in Example 1 except that the relative humidity was changed to 15%. The evaluation results are shown in Table 6. The alumina hydrate in the recording medium prepared in this Example had higher crystallinity, and thereby the ink absorbency was improved as shown in Table 6.

TABLE 6

|                                               | Evaluation Results in Example 11 |  |
|-----------------------------------------------|----------------------------------|--|
|                                               | Example 11                       |  |
| Crystallinity                                 | 20.0                             |  |
| BET specific surface area (m <sup>2</sup> /g) | 195                              |  |
| Pore volume (cm <sup>3</sup> /g)              | 0.56                             |  |
| Ink Absorbency                                | Good                             |  |
| Ink absorption rate                           | Good                             |  |
| Surface hardness                              | H                                |  |
| Cracking                                      | Good                             |  |

## 15

## EXAMPLES 12 to 15

Alumina hydrate liquid dispersions were prepared in the same manner as in Examples 1-4 except that the aging conditions and drying conditions for the alumina hydrate of boehmite structure were changed as shown in Table 7. The liquid dispersions were applied and dried respectively by means of a kiss-roll coater. The shearing stresses given to the liquid dispersions are shown in Table 7. The shearing stress was adjusted by changing the slit width and the extrusion pressure of the coating head. The amount of the coating was 7 g/m<sup>2</sup> in each Example. The coating was conducted at a rate of 0.8 m/s. The coated material was delivered without blowing drying air for one second after the coating application to thicken and set the coating by utilizing thixotropy of the coating liquid, and then it was dried for 25 seconds at 85° C. at a relative humidity of 35%.

Table 8 shows the results of the evaluation of the resulting recording medium.

TABLE 7

| Aging and Coating Conditions for Alumina hydrate |             |      |      |      |
|--------------------------------------------------|-------------|------|------|------|
|                                                  | Example No. |      |      |      |
|                                                  | 12          | 13   | 14   | 15   |
| pH before aging                                  | 6.3         | 6.6  | 6.3  | 6.5  |
| Aging temperature (° C.)                         | 35          | 38   | 40   | 33   |
| Aging period (days)                              | 16          | 12   | 15   | 17   |
| Aging apparatus                                  | Oven        | Oven | Oven | Oven |
| Crystallinity                                    | 16.0        | 45.2 | 52.5 | 30.0 |
| Shearing stress (N/m <sup>2</sup> )              | 0.2         | 10.8 | 19.8 | 0.3  |
| BET specific surface area (m <sup>2</sup> /g)    | 225         | 215  | 210  | 220  |
| Pore volume (cm <sup>3</sup> /g)                 | 0.70        | 0.71 | 0.71 | 0.70 |

TABLE 8

| Evaluation Results in Example 12-15           |             |      |      |      |
|-----------------------------------------------|-------------|------|------|------|
|                                               | Example No. |      |      |      |
|                                               | 12          | 13   | 14   | 15   |
| Crystallinity                                 | 16.5        | 45.3 | 52.6 | 28.6 |
| Parallelization degree                        | 1.6         | 1.8  | 2.6  | 1.7  |
| BET specific surface Area (m <sup>2</sup> /g) | 190         | 187  | 185  | 188  |
| Pore volume (cm <sup>3</sup> /g)              | 0.51        | 0.52 | 0.52 | 0.51 |
| Light fastness                                | Good        | Good | Good | Fair |
| Water fastness                                | Fair        | Good | Good | Good |
| Ink migration                                 | Good        | Good | Good | Good |

The present invention has the advantages listed below:

(1) A recording medium having higher ink absorbency, absorbing ink at a higher rate, and having a higher surface hardness is obtained by adjusting the crystallinity of alumina hydrate in the recording medium to be within in the specified range.

(2) A recording medium enabling higher circularity of printed dots and having higher gloss is obtained by adjusting the parallelization degree of alumina hydrate in the recording medium to be within the specified range.

(3) A printed matter having better light fastness, and water resistance, and being less likely to cause migration of ink is obtained by adjusting the crystallinity and the parallelization degree respectively to be within the specified ranges.

## 16

## What is claimed is:

1. A recording medium having a porous ink-receiving layer containing alumina hydrate having boehmite structure formed on a base material, said alumina hydrate having crystallinity ranging from 15 to 80.

2. The recording medium according to claim 1, wherein said alumina hydrate has crystallinity ranging from 20 to 70.

3. The recording medium according to claim 1, wherein said alumina hydrate is represented by the following formula:



where n is an integer of 0 to 3, m is a number of 0 to 10, and n and m are not both zero.

4. The recording medium according to claim 1, wherein said alumina hydrate has a particle size in a range of from 1 to 50 nm.

5. The recording medium according to claim 1, wherein said alumina hydrate has a pore volume ranging from 0.1 to 1.0 cm<sup>3</sup>/g.

6. The recording medium according to claim 1, wherein said alumina hydrate has a pore radius ranging from 2.0 to 20.0 nm.

7. The recording medium according to claim 1, wherein said ink-receiving layer contains a binder.

8. The recording medium according to claim 7, wherein a mixing weight ratio of said alumina hydrate to the binder is in a range of from 5:1 to 25:1.

9. The recording medium according to claim 7, wherein said binder is a material selected from the group consisting of polyvinyl alcohol, modified polyvinyl alcohol, starch, modified starch, gelatin, modified gelatin, casein, modified casein, gum arabic and cellulose derivative.

10. A process for producing the recording medium according to claim 1, comprising the steps of:

applying a liquid dispersion containing alumina hydrate having boehmite structure having crystallinity ranging from 15 to 80 on a base material; and drying the coated material at a relative humidity of 20 to 60% to obtain crystallinity of said alumina hydrate ranging from 15 to 80 in the recording medium.

11. A process for producing the recording medium according to claim 1, comprising the steps of:

applying a liquid dispersion containing alumina hydrate having boehmite structure having crystallinity of lower than 15 on a base material; and drying the coated material at a relative humidity of 10 to 20% to obtain crystallinity of said alumina hydrate ranging from 15 to 80 in said recording medium.

12. A process for producing the recording medium according to claim 1, comprising the steps of:

applying a liquid dispersion containing alumina hydrate having boehmite structure having crystallinity of lower than 15 on a base material; allowing the applied liquid dispersion to dry, whereby an ink-receiving layer is formed; and heating the coated material at a relative humidity of 10 to 20% to obtain crystallinity of said alumina hydrate ranging from 15 to 80 in said recording medium.

13. The recording medium according to claim 1, wherein said porous ink-receiving layer has a BET specific surface area in a range of from 20 to 450 m<sup>2</sup>/g.

14. A recording medium having a porous ink-receiving layer consisting essentially of alumina hydrate and a binder on a base material, wherein the alumina hydrate has boehmite structure and crystallinity ranging from 15 to 80.

17

15. The recording medium according to claim 14, wherein said alumina hydrate has crystallinity ranging from 20 to 70.

16. The recording medium according to claim 14, wherein said alumina hydrate is represented by the following formula:



where n is an integer of 0 to 3, m is a number of 0 to 10, and n and m are not both zero.

17. The recording medium according to claim 14, wherein said alumina hydrate has a particle size in a range of from 1 to 50 nm.

18. The recording medium according to claim 14, wherein said alumina hydrate has a pore volume ranging from 0.1 to 1.0 cm<sup>3</sup>/g.

19. The recording medium according to claim 14, wherein said alumina hydrate has a pore radius ranging from 2.0 to 20.0 nm.

18

20. The recording medium according to claim 14, wherein a mixing weight ratio of said alumina hydrate to the binder is in a range of from 5:1 to 25:1.

21. The recording medium according to claim 14, wherein said binder is a material selected from the group consisting of polyvinyl alcohol, modified polyvinyl alcohol, starch, modified starch, gelatin, modified gelatin, casein, modified casein, gum arabic and cellulose derivative.

22. The recording medium according to claim 14, wherein said porous ink-receiving layer has a BET specific surface area in a range of from 20 to 450 m<sup>2</sup>/g.

23. A recording medium for ink-jet recording having a porous ink-receiving layer containing alumina hydrate having boehmite structure formed on a base material, said alumina hydrate having crystallinity ranging from 15 to 80.

\* \* \* \* \*

UNITED STATES PATENT AND TRADEMARK OFFICE  
**CERTIFICATE OF CORRECTION**

PATENT NO. : 7,144,613 B2  
APPLICATION NO. : 08/974513  
DATED : December 5, 2006  
INVENTOR(S) : Takeo Eguchi et al.

Page 1 of 2

It is certified that error appears in the above-identified patent and that said Letters Patent is hereby corrected as shown below:

ON THE TITLE PAGE:

Item (56), References Cited, at U.S. Patent Documents, insert --5,445,868 8/1995  
Harasawa et al.--.

Item (56), References Cited, Other Publications, insert --Christoph et al., "The Crystal  
Structure of Boehmite", Clay and Clay Minerals, Vol. 27, No. 2, pp. 81-86, 1979--.

Item (56), References Cited, Foreign Patent Documents, insert --JP 6-262844 9/1994--.

COLUMN 1:

Line 26, "reproduction" should read --reproductions--.

COLUMN 9:

Line 36, "serves" should read --serve--.

Line 60, "or" should read --of--.

COLUMN 12:

Line 22, "by" should be deleted.

Lines 23-38 ("weight to obtain...as shown in Table 2.") should be deleted.

Line 53, "Condions" should read --Conditions--.

Line 67, "of 17%" should read --of 17% by weight to obtain an alumina liquid dispersion. Separately, polyvinyl alcohol (trade name: Gosenol NH18 (hereinafter referred to as "PVA"), Nippon Gosei Kagaku K.K.) was mixed with deionized water at a concentration of 17% by weight to obtain a PVA solution. The alumina liquid dispersion and the PVA solution were mixed at a mixing ratio of 18:1 to obtain a coating liquid. This coating liquid was applied onto a resin-coated paper sheet by means of an extrusion coater at a coating temperature of 100°C under shearing stress of 7.5 N/m<sup>2</sup> (75 dyn/cm<sup>2</sup>), and was delivered without blowing of drying air for one second to thicken and set the coating layer by utilizing thixotropy. Then the coating layer was dried for 30 seconds in an environment of relative humidity of 40% at a temperature shown in Table 2. The resulting recording medium was evaluated for the printing properties, etc. The evaluation results are shown in Table 2.--.

UNITED STATES PATENT AND TRADEMARK OFFICE  
**CERTIFICATE OF CORRECTION**

PATENT NO. : 7,144,613 B2  
APPLICATION NO. : 08/974513  
DATED : December 5, 2006  
INVENTOR(S) : Takeo Eguchi et al.

Page 2 of 2

It is certified that error appears in the above-identified patent and that said Letters Patent is hereby corrected as shown below:

COLUMN 15:

Line 61, "parellelization" should read --parallelization--.

Signed and Sealed this

Thirtieth Day of October, 2007

A handwritten signature in black ink, appearing to read "Jon W. Dudas", is centered within a dotted rectangular border.

JON W. DUDAS  
*Director of the United States Patent and Trademark Office*